

May 4, 1954

L. H. JENNINGS

2,677,151

METHOD OF CASTING WAX SLABS

Filed Nov. 3, 1951



INVENTOR.  
Leon H. Jennings  
BY  
Raymond J. Rubbia  
ATTORNEY

## UNITED STATES PATENT OFFICE

2,677,151

## METHOD OF CASTING WAX SLABS

Leon H. Jennings, Beaumont, Tex., assignor to  
Socony-Vacuum Oil Company, Incorporated,  
New York, N. Y., a corporation of New York

Application November 3, 1951; Serial No. 254,682

5 Claims. (Cl. 18—58)

1

This invention is directed to a method for the production of paraffin waxes in slab form.

One normal form in which paraffin wax is prepared for distribution to the trade is in a slab or cake weighing about eleven pounds, which is about 18½ inches by 11½ inches and about 1½ inches thick.

Usually these cakes or slabs are prepared by a batch method, using an arrangement of alternating open-top molds and internally water-cooled dividers which are assembled upon side-rods and held together by end-pressure on the assembly. The melted wax is poured into the trough formed by the top of the assembly and fills the mold and is cooled therein by water passed through the dividers. After cooling, the wax remaining above the top of the molds is cut or scraped off, the assembly is loosened and the cakes are removed. This method involves a very considerable amount of hand labor and handling of cakes.

There has now been applied to this problem a process of continuous molding in pans adapted from a somewhat analogous industry.

The object of this invention is to provide a proper control for this operation, as will be explained in detail herein.

In order to understand the operation, reference is now made to the drawing which accompanies and is made a part of this specification. This drawing shows, in highly diagrammatic form, the process of slab casting. A series of pans 1, 1, 1, etc., are carried upon a chain 2, 2, 2, etc. These pans are of the proper size for the desired wax slabs, and are closely spaced upon the side chains and arranged in transverse gangs of six pans, side by side. At the left hand end of the lowest pass of the chain, they pass under a depositor, consisting of a hopper 3 and a transverse series of piston type feeders 4, whereby a measured amount of molten wax is withdrawn from hopper 3 and deposited in each pan. Passing to the right, the pans enter into a cooled enclosure designated by dotted lines 5, wherein they are blasted with cooling air to bring about solidification of the wax. The pans are led through a series of horizontal passes in the cooler (14 passes in one installation), only four being shown in the diagram for purposes of simplicity. The chain and conveyor system is so arranged that the pans remain in an upright and horizontal position, without disturbance of the wax enough to cause distortion of the cake surface, while passing through the cooler. The cooler is fed with cold air, supplied from cooling coils located at

2

one side of the cooler enclosure and blown transversely therethrough.

Emerging from the cooler 5, at the upper left hand end in the diagram, the pans are passed through an upsetting turn and put into an upside down position in the chain pass indicated by 6. This upsetting results in the dropping of the wax slab 7 which through the agency of conveyors 8 and 9, associated with the upsetting or discharge mechanism, is finally placed in position on discharge conveyor 11 by which it is withdrawn laterally from the slabbing machine. The pans 1 are then righted, and prior to loading by distributor 4 are passed over a preheater 12 which heats the pans slightly before they are filled.

The normal operation is to maintain the air temperature and air rate in the cooling chamber and to vary the rate of cooling when necessary by varying the conveyor speed and hence the residence time of the pans within the cooling chamber.

This equipment is essentially the same as is used in slabbing chocolate, etc., and as such forms no part of this invention.

The present requirements for cake wax, particularly paraffin require careful attention to appearance. The surface of the cake must be clean and free from ripples and bumps and the cake should show no lamination nor broken edges. Even more important, its surfaces should be cleanly formed and as nearly as possible at right angles to each other for economy and ease in packaging. This last requires that the pans be formed with a very minimum of taper or "draft," and gives rise to a problem in cleanly dumping the pans. These and other considerations make it necessary to closely control the operation as to temperature.

First, as to the loading of the pans. Obviously this temperature should be near to the melting point of the wax to save cooling load. It cannot be too low. If too low, it is found that films of cooler wax form next to the bottom and sides of the pan, the cake refuses to dump cleanly regardless of final temperature, and also trouble is had with cake lamination, frequently causing scaling of the discharged cake.

I have found that the proper temperature at which the wax, regardless of its melting point, must be loaded to the pan is at 20° F. above its ASTM melting point. (ASTM melting point is the melting point as determined by ASTM Method D87-42, specified by the American Society for Testing Materials, also designated as ASA Method No. Z 11.4-1942 and API No. 513-42.)

The temperature of loading should not vary more than minus 2° F. from the specified level.

The final temperature to which the wax should be cooled is also a matter of major importance. It should not only be low enough to permit clean dumping of the wax cake or slab, but since the slab is cooled from the outside and the center of the cake is warmest, the cake or slab should not contain enough residual heat to soften up and lose shape or block (adhere to adjacent slabs), after removal from the pans. I have found that this condition can be fulfilled by cooling the cake until its center temperature is at least about 30° F. below the ASTM melting point. This temperature can be taken by inserting thermometers from time to time in individual cakes as a check, but in actual operating practise is handled by holding the temperature and rate of cooling air flow constant and controlling the length of time of exposure of the slabs to this cooling.

The rate of cooling is also of importance. Shock chilling is not a factor since I have found that the air may be as cold as practicable, even 5° F., so long as even air flow and exposure of the slabs thereto is provided. In some instances it may be necessary to protect a portion of the cooling cycle, such as the portion found at the lower right hand end of the diagram, from too vigorous air flow. The object is to secure a uniform rate of cooling throughout the entire chain pass. With such uniform cooling, although the center of the slab will of course cool more slowly than the outside, fairly uniform conditions within the slab will be gotten if the time of cooling is proper. This of course depends not so much upon the temperature of the cooling air as it does upon the nature of the wax itself as a heat transfer medium. I have found that for wax slabs of conventional size, cooled from at least 20° F. above their ASTM melting point to at least 30° F. below their ASTM melting point, the time of cooling should be of the order of 135 to 150 minutes. Expressed in rate, the cooling should be from not less than about 2 minutes per degree F. to not more than about 3.5 minutes per degree F.

Several examples of successful operation are as follows:

Table

| ASTM M. P.<br>of Wax | Loading<br>Temp.<br>° F. | Discharge<br>Temp.<br>° F. | Cooling Time |           | 50 |
|----------------------|--------------------------|----------------------------|--------------|-----------|----|
|                      |                          |                            | Minutes      | Min./° F. |    |
| 125 M. P.            | 145                      | 80                         | 150          | 2.3       |    |
| 135 M. P.            | 155-160                  | 90-95                      | 135          | 2.08      | 51 |

In these operations, clean, sharply formed paraffin wax slabs, without internal laminations and without broken edges, "pickouts," or other evidence of poor dumping were made, and dumped with ease. Neither did the slabs so made show any evidence of blocking or deformation after being removed from the slabbing machine.

Attempts to operate this machine without attention to these controls resulted in paraffin slabs

65

which were not marketable because of the various defects mentioned.

I claim:

1. In the method of converting paraffin wax into clean, sharply-formed paraffin wax slabs, substantially without internal laminations and broken edges, which includes depositing paraffin wax in a mold pan, moving the pan through a cooling chamber and discharging a solidified wax slab from the pan, the improvement which comprises loading the wax into the pan at a temperature not less than about 20° F. above its ASTM melting point, cooling the wax slowly to a temperature at the center of the slab which is not above about 30° F. below the ASTM melting point of the wax, and dumping the slab.

2. In the method of converting paraffin wax into clean, sharply-formed paraffin wax slabs, substantially without internal laminations and broken edges, which includes depositing paraffin wax in a mold pan, moving the pan through a cooling chamber and discharging a solidified wax slab from the pan, the improvement which comprises loading the wax into the pan at a temperature not less than about 20° F. above its ASTM melting point, cooling the wax slowly during a time of from about 135 to about 150 minutes to a temperature at the center of the slab which is not above about 30° F. below the ASTM melting point of the wax, and dumping the slab.

3. In the method of converting paraffin wax into clean, sharply-formed paraffin wax slabs, substantially without internal laminations and broken edges, which includes depositing paraffin wax in a mold pan, moving the pan through a cooling chamber and discharging a solidified wax slab from the pan, the improvement which comprises loading the wax into the pan at a temperature not less than about 20° F. above its ASTM melting point, cooling the wax slowly at a rate ranging from not less than about 2 minutes per degree F. to not more than about 3.5 minutes per degree F. to a temperature at the center of the slab which is not above about 30° F. below the ASTM melting point of the wax, and dumping the slab.

4. A method as defined in claim 1 wherein a chain of mold pans are conveyed continuously through the wax depositing station, thence through the cooling chamber and thence through the slab dumping station.

5. A method as defined in claim 2 wherein a chain of mold pans are conveyed continuously through the wax depositing station, thence through the cooling chamber and thence through the slab dumping station.

## References Cited in the file of this patent

## UNITED STATES PATENTS

| Number    | Name    | Date          |
|-----------|---------|---------------|
| 22,921    | Leonard | Feb. 8, 1859  |
| 1,658,062 | Sprague | Feb. 7, 1928  |
| 2,476,710 | Eaton   | July 19, 1949 |